

Patented Nov. 15, 1927.

1,649,100

# UNITED STATES PATENT OFFICE.

FRANKLIN NORRIS CHILDS, OF DANVILLE, PENNSYLVANIA.

## COMPOUND FOR FILLING HOLES IN CAST IRON.

No Drawing.

Application filed December 9, 1924. Serial No. 754,855.

This invention relates to a compound in the form of paste, adapted to be used for filling up the holes and defects in iron castings, preparatory to enameling the same.

5 It is a well-known fact that no matter how carefully and skillfully the casting operation is performed, certain holes or depressions will be formed to a greater or less extent in the surface of the casting due to 10 accumulated particles of sand or slag, so that it is often impossible to cover them sufficiently by enamel alone to secure a smooth and uniform surface.

The object of the present invention is to 15 provide a compound which may be applied to the casting in much the same manner as putty is applied to holes or defects in wood surfaces preparatory to painting or varnishing the same, and it is especially important 20 that the compound be so constituted that it will not be adversely affected by the extreme heat necessary to bake the enamel, and will, in fact, form a union with the casting so as to make, for all intents and purposes, a 25 solidified whole.

The body of the composition, which constitutes the subject matter of my invention, consists of fine iron filings. These filings are made preferably from soft pig iron after 30 the temper has been removed therefrom, so as to make it easily reducible. These filings are then passed through a fine sieve, and are then mixed with a sufficient quantity of 35 a solution of sulphate of magnesia in water to form a compound of about the same consistency as putty. The solution of sulphate of magnesia is composed of approximately one part of sulphate of magnesia to twelve 40 parts of water. The water acts as a solvent for the sulphate of magnesia, and the solution acts as a vehicle for the iron filings so as to form a compound which may be easily molded and worked into the holes in the casting, leaving a smooth surface to which 45 the enamel may be applied.

The compound can be kept indefinitely by placing it in air tight metallic tubes or other air tight containers; and in case it should become dry, water may be applied to restore 50 it to proper consistency.

The usual method of applying the enamel

is by spraying it on the surface of the casting after the latter has been rendered smooth and uniform by the use of the compound. The enamel is then baked at a temperature 55 of 1200° to 1250° F.

Cast iron surfaces after they have been treated in this manner and enameled will be perfectly smooth, and no defects in the castings will be discernible. The sulphate 60 of magnesia serves as a cement to hold the filings in place until the first coat of enamel is applied, and also replaces a certain amount of enamel which is burned up in the baking process. The water serves to give 65 the compound a pasty consistency so that it may be easily applied. The iron filings, together with the sulphate of magnesia, upon the application of heat during the baking process, causes such a union of the compound with the casting as to make an integral 70 whole, resulting in a smooth, even surface, which can not be obtained by the use of enamel alone. I am, however, unable to state whether or not the compound actually 75 forms a chemical combination with the casting.

While I have described approximately the proportions of the several materials which are believed to be the most desirable to use, 80 it is apparent that these proportions may be varied between wide limits without materially affecting the results.

What is claimed is:

1. A compound for the purpose described, 85 consisting of finely divided particles of iron mixed with a quantity of sulphate of magnesia dissolved in water.

2. A plastic compound, consisting of finely divided particles of iron mixed with a 90 sufficient quantity of sulphate of magnesia dissolved in water to form a stiff paste.

3. A compound for the purpose described, 95 consisting of soft iron filings mixed with a sufficient quantity of a solution of sulphate of magnesia in water to form a stiff paste, said solution being approximately in the proportion of one part sulphate of magnesia to twelve parts water.

In testimony, that I claim the foregoing as 100 my own, I have hereto affixed my signature.

FRANKLIN NORRIS CHILDS.